

# United States Patent

[11] 3,572,042

|      |           |                                                                          |           |         |                      |        |
|------|-----------|--------------------------------------------------------------------------|-----------|---------|----------------------|--------|
| [72] | Inventor  | Thorndyke Roe, Jr.<br>Oxnard, Calif.                                     | 3,236,671 | 2/1966  | Dybalski et al. .... | 61/36X |
| [21] | Appl. No. | 864,222                                                                  | 3,252,290 | 5/1966  | Gagle et al. ....    | 61/36  |
| [22] | Filed     | Oct. 6, 1969                                                             | 3,312,069 | 4/1967  | Jorda.....           | 61/36X |
| [45] | Patented  | Mar. 23, 1971                                                            | 3,332,245 | 7/1967  | Caron.....           | 61/36  |
| [73] | Assignee  | The United States of America as represented by the Secretary of the Navy | 3,359,738 | 12/1967 | Dybalski et al. .... | 61/36X |
|      |           |                                                                          | 3,446,027 | 5/1969  | Meijer.....          | 61/1X  |

Primary Examiner—Stephen J. Novosad  
Attorneys—R. S. Sciascia and Paul N. Critchlow

[54] **PROCESS FOR FORMING A PLASTIC FILL SHEET ON OCEAN FLOOR SILT**  
2 Claims, No Drawings

|      |                                  |                                               |
|------|----------------------------------|-----------------------------------------------|
| [52] | U.S. Cl.                         | 61/36,<br>61/7                                |
| [51] | Int. Cl.                         | E02b 3/12,<br>E02b 29/06                      |
| [50] | Field of Search                  | 61/36, 1,<br>35; 116/295, 0.5; 260/33.4, 31.8 |
| [56] | References Cited                 |                                               |
|      | UNITED STATES PATENTS            |                                               |
|      | 2,615,307 10/1952 Kjellman ..... | 61/36X                                        |

**ABSTRACT:** A resin solution is fed through an extrusion head disposed underwater and in close proximity to the sediment of the ocean floor. The solution is formed of a sea water insoluble resin-plasticizer system dissolved in a sea water insoluble solvent, the resin-plasticizer system of the solution having a relatively high specific gravity greater than 1.0 so that, when the system precipitates in the sea water, it drops onto the sediment. Preferably, the extrusion head is moved along at a controlled rate to form a continuous sheet of a desired thickness.

**PROCESS FOR FORMING A PLASTIC FILL SHEET ON  
OCEAN FLOOR SILT**

**BACKGROUND OF THE INVENTION**

The present invention relates to processes or techniques for settling loose or suspended sea floor sediment to improve underwater visibility. In particular, it relates to plastic films adapted for these purposes.

In many underwater operations, such as salvage operations or the more recently conducted Sealab tests, it is highly desirable to provide maximum visibility and, of course, loose sediment, such as is commonly found on the ocean floor, seriously restricts visibility when it is stirred into a suspended state. In such situations, it becomes necessary to wait until the sediment again settles and, since time is a critical factor in any underwater operations, the waiting period presents real problems. Various methods, such as the use of flocculating agents to settle the suspended sediments, have been attempted. However, although these agents are somewhat effective, once the settled material is disturbed, the waiting period still is required.

Another problem frequently experienced in underwater operations arises when the operator accidentally drops a hand tool or other oceanographic instruments onto the heavy layer of silt deposited on the ocean floor. Due to the weight of these objects, they become deeply imbedded in the silt and frequently are lost or, at least, require a substantial recovery time.

**BRIEF SUMMARY OF THE INVENTION**

The present invention minimizes the foregoing difficulties by forming a sediment-blanketing plastic film sheet directly on the loose sea floor sediment. To form the sheet, a solution formed of a sea water insoluble resin-plasticizer system dissolved in a sea water miscible solvent is extruded from a container through a submerged extrusion head directly onto the sediment. The resin system has a relatively high specific gravity so that the precipitate drops through the sea water onto the sediment and, to provide a continuous sheet, the extrusion head simply is moved along the sediment at a controlled rate. Typical formulations for the solution are set forth in the ensuing detailed description.

As already indicated, a primary object of the invention is to provide a means for forming continuous plastic sheet directly on loose sea floor sediment.

A related object is to form a sheet which becomes a flexible platform capable of supporting light loads as well as preventing loss of items accidentally dropped during underwater operations.

Another object is to form a sediment-blanketing sheet the strength of which increases with time.

Other objects, advantages and novel features of the invention will become apparent from the following detailed description of the invention.

**DETAILED DESCRIPTION OF THE INVENTION**

The apparatus used in carrying out the present process is not part of the present invention and, since it can be provided in a variety of well-known manners, it would seem that the present invention is capable of being readily understood without the need of special drawings or illustrations. In general, the apparatus may include a reservoir for containing the film-forming solution and the reservoir should be connected to a dispensing head equipped with a shutoff valve and an extrusion slit. In carrying out the process the reservoir is filled with the solution and then submerged into close proximity with the sediment on the ocean floor. The valve is opened and the solution is permitted to escape through the extrusion slit. In actual practice, it will be found that some means for pressurizing the solution greatly facilitates the escape and, for this purpose, the reservoir may be coupled by a conduit to a pneumatic source or, if desired, a flexible or collapsible bag-type reservoir can be employed to make use of the compres-

sive forces of undersea pressures to facilitate removal or extrusion of the plastic film-forming substances. Pressure is desirable since, as will be explained, the resin in the solution commences to solidify and precipitate immediately upon being exposed to the sea water environment.

With regard to the film-forming solution, the following is a typical or representative formulation which, in practice, has been found to provide a continuous flexible plastic film capable of covering the ocean floor sediment and preventing the sediment from becoming disturbed and suspended in the sea water. Also, this plastic film was found to have a strength sufficient to support light loads and a strength which increased with deposit time:

|    |                            |        |
|----|----------------------------|--------|
| 15 | Polyvinyl butyral resin    | 2 lb.  |
| 20 | 2-(2-ethoxyethoxy) ethanol | 5 gal. |
| 25 | Chlorinated biphenyls      | 26 lb. |
| 30 | Dibutyl phthalate          | 18 lb. |

If desired, a dye such as Rhodamine B can be included in the formulation to render the deposited plastic sheet readily visible to the operator.

It is highly essential in formulating the solution to use a resin-plasticizer system which has a specific gravity greater than 1.0 and, preferably, a significantly greater than 1.0 so as to minimize any suspension of the plastic in the water. In other words, the precipitated resin plastic system must have a unit volume weight high enough to promote its dropping from the extrusion head onto the sea floor sediment. In the foregoing formulation, the plasticizer is incorporated to adequately increase the unit volume weight of the system, although, of course, the plasticizer also performs its customary function of rendering the film flexible.

The other significant factor in the formulation is the use of a solvent which itself is miscible and preferably soluble in sea water. Consequently, when the solution initially is exposed to the sea water, the solvent commences to dissolve in the sea water permitting the resin system to precipitate out in a desired manner. The initial film formed by the precipitation is sufficiently cohesive to provide a continuous sheet although, as will be apparent, the toughness or strength of the sheet will not be achieved until the solvent has completely dissolved in the water. It is for this reason that the strength of the film increases with time.

A variety of resins, solvents and plasticizers can be employed to provide the desired sediment blanket. For example, it has been found that other resins, such as acrylonitrile-styrene; polyvinyl chloride-acetate, and polyvinylidene chloride (saran), can be substituted. The two plasticizers identified in the foregoing formulation appear to be best for the present purposes although it certainly is conceivable that other plasticizers would perform in the desired manner. Other representative solvents that can be used in lieu of the solvent identified in the formation are chloroethanol, dimethyl formamide and dimethyl sulfoxide. The substitute materials can be incorporated in approximately the same percentages used in the preferred formulation.

In any of these formulations, it is desirable to use sufficient solvent to permit a relatively free flow of the solution through the extrusion head. Too rapid formulation of the precipitate interferes with the extrusion and promotes clogging of the extrusion head. Other factors involved in the actual application of the film should be readily resolvable simply by trial and error procedures. For example, the thickness of the deposited film can be controlled by the rate of moving the extrusion head over the ocean floor.

Obviously many modifications and variations of the present invention are possible in the light of the above teachings. It is therefore to be understood that within the scope of the appended claims the invention may be practiced otherwise than as specifically described.

I claim:

1. A process of depositing a sediment-blanketing plastic film sheet directly onto loose sea floor sediment comprising:  
 forming a solution of a sea water insoluble resin-plasticizer system dissolved in a sea water miscible solvent;  
 extruding the solution from a container through a submerged extrusion head disposed directly over and in close proximity to said sediment;  
 moving said extrusion head at a rate sufficient to permit said resin-plasticizer system to precipitate in the sea water and drop in a continuous sheet onto the sediment; and  
 said resin-plasticizer system having a specific gravity greater

than 1.0 whereby the precipitate drops through the sea water onto the sediment.

2. The process of claim 1 wherein said solution consists essentially of the following formulation as expressed in parts by weight:

|                            |    |
|----------------------------|----|
| polyvinyl butyral resin    | 2  |
| 2-(2-ethoxyethoxy) ethanol | 40 |
| chlorinated biphenyls      | 26 |
| dibutyl phthalate          | 18 |